

Jan. 5, 1960

M. A. MILLER

2,920,018

ANODIZING PROCESS AND SYSTEM

Filed April 22, 1957

Fig. 1



Fig. 2



Fig. 4



Fig. 3



INVENTOR:  
Myron A. Miller

By L. Mylly & Roston  
Attorneys

1

2,920,018

## ANODIZING PROCESS AND SYSTEM

Myron A. Miller, North Hollywood, Calif., assignor to  
Electro-Chem Manufacturing Co., Inc., Los Angeles,  
Calif.

Application April 22, 1957, Serial No. 654,330

5 Claims. (Cl. 204—56)

The present invention relates to an improved anodizing process and apparatus for producing inorganic oxide coatings on metallic bodies, such as aluminum and other materials capable of being anodized.

In recent years, certain materials capable of acquiring anodic coatings have come into widespread use. Such coatings are formed on the particular materials by an electro-chemical modification of its surface to become an integral part of the material itself. The resulting coating is highly resistant to corrosion and it is non-reactive.

The electro-chemical modification of the material surface referred to above is achieved by means of a process known as anodizing. In the anodizing process, the work-piece is immersed in a bath of a suitable electrolyte, and it forms the anode of an electric circuit through which a current is passed. Anodizing has been applied most successfully to pure aluminum and certain aluminum alloys, and the process and apparatus of the present invention will be described in conjunction with these materials. The technique, however, has also been applied to zinc and magnesium, and to other materials. It will be evident as the description proceeds that the apparatus and process of the invention are applicable to any material capable of acquiring an anodized coating.

The tendency of an aluminum body to form an oxide film or coating when the body is made the anode of an electrolytic cell, has been known for many years. The fact that this oxide coating exhibits uni-directional current characteristics has also been known for a long time. However, it was only within the last 20 years that processes have been devised for producing relatively thick and commercially usable anodic coatings for corrosion protection. Also, it is only within the last few years that anodizing processes have been brought within the realm of commercial practicability.

The original anodizing process, which was developed over 20 years ago, utilizes a chromic acid bath as the electrolyte. This original process is still in use today in some countries, notably England. In the United States, however, the original process has been superseded to a large extent by processes using sulphuric or oxalic acid baths, or a combination of the two acids.

The characteristics of the anodic coating are largely determined by the particular electrolyte that is used. For example, when an electrolyte solution of boric acid is used, the resulting anodic oxide coatings are substantially indissoluble in the electrolyte. This electrolytic solution produces thin, impervious oxide coatings as are required in electrolytic condensers and the like. However, these particular coatings are not particularly corrosion or abrasion resistant.

On the other hand, when the electrolyte is sulphuric, oxalic, or chromic acids, the resulting oxide coating is continually being dissolved by the electrolyte as the process is being carried out. This results in the production of a relatively thick, but porous, coating.

The anodic coatings which result from the use of sul-

2

phuric acid, or the other acids described in the immediately preceding paragraph, afford high protection from corrosion and they are highly resistant to abrasion. However, as noted, these coatings are formed in electrolytes which exert an appreciable dissolving action on the coating as it is being formed. This counteracting solvent action produces problems which will be discussed subsequently. Moreover, the coatings are often relatively soft and unduly porous when formed by most of the prior art processes. The desired end in this area is to produce an anodic coating that is thick, hard and not unduly porous.

One known prior art anodizing process uses a 3% solution of chromic acid as the electrolyte bath. The bath is maintained at 40°—45° C. by means of refrigeration cooling coils while the process is being carried out. Such cooling coils are required because of the liberation of heat by the process and the need to prevent undue heating of the electrolyte with corresponding increased dissolution of the anodic film by the electrolyte. At the beginning of the operation, the voltage is held at around 40 volts, and this voltage is maintained for the first 15 minutes. The voltage is then raised to 50 volts so as to maintain a constant current flow through the system as the oxide anodic layer builds up and increase the anode resistance. The total time required in this prior art process is of the order of one hour, and the current density ranges from 2.5—4 amps./sq. ft. Films of the order .1—.2 thousandths of an inch can be formed by this prior art process. The limitation on the thickness of the anodic layer or film resides in the fact that a particular current flow must be maintained in order that the layer may be built up faster than it is being dissolved by the electrolyte. However, as indicated above, the voltage must be continually increased to maintain this constant current as the essentially non-conductive surface layer is built up on the anode surface. This increased voltage increases the temperature at the anode surface which increases the reaction ability of the electrolyte with the layer. The limit of thickness of the layer is reached when the current flow and resulting temperature at the anode reaches a limit such that an increase in voltage to maintain a particular current flow produces a greater dissolving effect in the electrolyte, so that such voltage increase results in no increase in layer thickness.

A more recent process has been developed. This latter process uses sulphuric acid as an electrolyte, and it is capable of producing hard transparent coatings on aluminum which are materially thicker than those produced by the process described above.

After the anodizing operation, the resulting oxide coating is usually treated by boiling water which transforms the anodic aluminum oxide film ( $Al_2O_3$ ) into aluminum anhydrate. The result is a reduction in film porosity and an improvement in its resistance to corrosion. This latter operation must be carefully controlled to obtain a uniform product.

In general, and as mentioned briefly above, in the production of anodic coatings the electric current through the electrolyte tends to form the anodic film, whereas the electrolyte itself tends to counteract the action of the current and dissolve the film. An increase in the temperature of the electrolyte tends to increase its attack on the anodic film. Also, as previously mentioned, the reaction tends to generate heat and refrigerating coils are usually required to maintain the temperature of the bath at a relatively low temperature so as to reduce the tendency of the electrolyte to dissolve the oxide coating. The electric current passed through the electrolyte must penetrate the anodized oxide film to the conductive anode body. This is because anodizing takes place between the

base surface of the anode and the anodized oxide film. This is different from electrodepositing in which a conductive layer is built up on the base electrode and the electrodepositing action takes place on the surface of the deposited layer. Therefore, problems are encountered in anodizing processes that are not met in electrodepositing.

For example, the anodic film is a good dielectric and, therefore, as the film is built up by the anodizing process, the electric resistance of the anode increases. This is why the voltage, as indicated previously, has to be increased as the operation progresses so as to maintain the constant current flow which is essential to build up the desired film. However, as noted, the increase of voltage results in an increase in the amount of heat at the anode surface. This in turn increases the rate at which the coating is dissolved by the electrolyte. A limiting film increase is reached, therefore, when the rate of chemical dissolution of the film by the electrolyte is equal to the rate of film growth.

Therefore, to produce a thick, hard anodized film it is necessary to increase current density in some manner without an accompanying excessive increase in the temperature of the anode surface.

There also is a problem of initial passivity of the anode, due to polarization. This latter problem is of more significance when it is attempted to anodize highly alloyed aluminum materials. The phenomenon of anode polarization is well known to the art. Anode polarization produces a tendency for the workpiece to "burn" and be destroyed or severely damaged during the anodizing process. Moreover, the ability of any anodizing process to form a thick and hard anodic film is materially reduced by anode polarization.

Some of the problems outlined in the preceding paragraphs have been solved to some extent by superimposing an alternating current on the direct anodizing current which is passed through the anode formed by the workpiece and through the electrolyte. The superimposed alternating current is in the form of a ripple on the direct anodizing current, and it does serve to overcome the adverse effects of anode polarization to some extent. Also, the use of the superimposed alternating current does permit higher current densities to be used for an increase in speed in the work cycle which results in harder and thicker coatings than those produced by the previous methods.

The use of the superimposed alternating current, as noted above, results in the production of a harder and thicker anodic coating than those previously attainable. However, the provision of the superimposed alternating current on the direct anodizing current requires relatively complicated, expensive and inflexible circuitry. Also, this superimposing of the alternating current does not solve the problem of heating at the anode surface which occurs, as noted above, when the current density is increased. As pointed out, this heating of the anode surface is a limitation on the thickness and hardness to which an anodizing film can be built up on the workpiece.

In the process of the present invention, the actual current flow through the anodizing apparatus is pulsed. This pulsing of the entire anodizing current not only overcomes the anode polarization problems described above, but it also provides a cooling period between each interval of current flow.

The anode cooling effect provided by the pulsing action of the present invention is not attainable by refrigeration cooling coils in the electrolyte. There is a limit to the extent to which the cooling coils can reduce the temperature of the electrolyte and yet permit the electrolyte to carry out its electro-chemical function in the anodizing process. However, even though the temperature of the electrolyte has been reduced to its absolute minimum limit for satisfactory electro-chemical action by the cooling coils, there is still excessive heat developed at the

anode surface. As described above, this heat increases the attack of the electrolyte on the anode which renders the anodic film soft and porous, and which also sets a limit to the thickness with which the anodic film can be built up.

The pulsing of the anode current in accordance with the present invention provides a direct cooling at the anode surface. This permits higher current densities to be used without concomitantly excessively increasing the reaction of the attack of the electrolyte on the anodic film. Therefore, the direct result is the production of thicker and harder anodic films than those produced by the prior art processes. The invention provides, therefore, an improved and simplified anodizing process which results in the production of relatively thick and hard anodized films, and in which such production is carried out in a quicker work cycle than that required by the prior art processes.

The invention also provides improved apparatus for carrying out the pulsating anodizing action of the inventive process. The apparatus is relatively simple and inexpensive to construct, and it is capable of easy and fool-proof operation even in the hands of an inexperienced workman.

Further advantages and features of the process and apparatus of the invention will be evident from the following description, when the description is considered in conjunction with the accompanying drawings in which:

Figure 1 is a schematic representation of apparatus constituting an embodiment of the present invention, and this representation shows mostly in block form various components which are suitable for carrying out the improved process of the invention;

Figure 2 is a circuit diagram of appropriate circuitry for the components shown in block form in Figure 1; and

Figures 3 and 4 are series of curves showing the various electrical signals and pulses that are produced in the apparatus of Figures 1 and 2, and which are used for carrying out the process of the invention.

The apparatus of Figure 1 includes an anodizing bath 10 of usual construction. This bath, for example, may be lined with a lead lining 11, and the lead lining constitutes in known manner the cathode for the anodizing process. A series of refrigeration cooling coils 12 are wound about the interior of the bath 10 adjacent the lining 11. These coils have a refrigerant passing through them from any suitable refrigerating apparatus. Most commercially available refrigerators are suitable for the purpose, and it is believed unnecessary to show or describe the details of a typical refrigeration unit. The use of refrigeration coils in the electrolyte of an anodizing bath per se is known.

The bath 10 is intended to hold a suitable electrolyte for anodizing purposes in electrical contact with the lead lining 11. The workpiece to be anodized is indicated as 14, and this workpiece is suspended by any suitable bracket means (not shown) in the electrolyte contained in the bath 10. Although anodizing is usually carried out on aluminum bodies and bodies composed of aluminum alloys, other materials also are susceptible to anodizing. For example, as noted above, bodies composed of magnesium and zinc, and other materials, have been successfully anodized.

The electrical components of the apparatus shown in Figure 1 include a source of alternating current 15. This source may be the usual domestic 115-volt, 60-cycle alternating current mains. The voltage from the source 15 is introduced to a phase-shifting circuit 16, and this circuit is coupled to a pulsing circuit 18. The pulsing circuit 18 is connected between the control grid and cathode of a gaseous discharge tube 20.

The discharge tube 20 may be of the type presently referred to as a thyratron, or an ignitron, although any other suitable known type of discharge tube can be used. The anode of the discharge tube 20 is connected to one side of the secondary winding of a transformer 22, and

the other side of this winding is connected to the lining 11 of the anodizing bath 10. The cathode of the tube 20 is connected to the workpiece 14 to be anodized over the indicated ground connection. A pair of output terminals 25 are included in these connections. As mentioned above, the workpiece 14 forms the anode in the electrolyte and the metal lining 11 of the bath 10 forms the cathode. The primary winding of the transformer 22 is connected to a source of alternating current 24 which may have the same characteristics as the source 15.

In a manner to be described in detail subsequently, the pulsing circuit 18 produces triggering pulses for the gas discharge tube 20. The phase shifting circuit 16 is manually controllable, so that the discharge tube 20 may be triggered at any point on the positive cycle of its anode voltage, as supplied from the source 24. By the control of the triggering of the gas tube 20, discrete uni-directional current pulses are established through the secondary of the transformer 22, and these pulses flow to the anode 14 through the electrolyte in the bath 10 from the cathode formed by the lining 11 of the tank enclosing that bath. Of course, a separate cathode immersed in the bath could be used. The resulting current pulses flowing through the electrolyte can be controlled as to amplitude and as to their individual duration by the control of the phase shifting circuit 16. The most satisfactory operation is obtained when the current pulses have a relatively large amplitude for high current density, and when there is a relatively long interval between each successive pulse for adequate cooling.

In a particular application of the process of the invention, the following conditions were present:

|                                                        |                                                         |
|--------------------------------------------------------|---------------------------------------------------------|
| Workpiece 14                                           | Aluminum.                                               |
| Electrolyte                                            | Sulphuric acid 11% by weight. Oxalic acid 1% by weight. |
| Electrolyte temperature                                | 38°-42° Fahrenheit.                                     |
| Current density                                        | 200 amps. per sq. foot.                                 |
| Anodizing time                                         | 10 minutes.                                             |
| Film thickness                                         | .002-.0035 inch.                                        |
| Current pulse duration (percentage of complete cycle). | 25%.                                                    |

As shown in Figure 2, the phase shifting circuit 16 includes a transformer 50 whose primary winding is connected to the alternating current source 15. A variable resistor 52 and a capacitor 54 are connected in series across the secondary winding of the transformer. A capacitor 56 is connected from the common junction of the resistor 52 and the capacitor 54 to the cathode of a diode 58. A resistor 60 is connected between the cathode of the diode 58 and ground, and a capacitor 62 is connected to the grounded end of the resistor 60 and to the center tap of the secondary winding of the transformer 50.

The anode of the diode 58 is connected to the control grid of a pentode 64. The cathode of the pentode is grounded, and its anode is connected to one terminal of a resistor 66. The suppressor electrode of the pentode 64 is connected to its cathode, and the screen electrode is connected to one terminal of a resistor 68. A grounded by-passing capacitor 70 is connected to the screen electrode. The other terminal of the resistor 66 and of the resistor 68 are both connected to the movable tap of a potentiometer 72. This potentiometer is connected in the output circuit of a usual power supply which will be described and which supplies positive unidirectional exciting potentials to the pentode 64.

A capacitor 74 is coupled between the anode of the pentode 64 and the control grid of the gas discharge tube 20 referred to previously. As noted above, the anode of the tube 20 is connected to one side of the secondary winding of the transformer 22, and the cathode of the tube is grounded. The output terminals 25, as described above, are connected to the other side of the

secondary winding of the transformer 22 and to ground. These terminals, as described, are connected to the anode 14 and to the lining 11 of the bath 10.

The power supply includes a usual power transformer 76 whose primary winding is connected to the alternating current source. The secondary winding 77 of the transformer 76 is connected to the anodes of a full-wave rectifier tube 78, and the center tap of the secondary winding is grounded. The transformer 76 also includes a filament winding 79, and the filament winding is connected to the filament of the rectifier tube 78. The center tap of the filament winding 79 is connected to one side of a choke coil 80, and the other side of the choke coil 80 is connected to one of the fixed contacts of the potentiometer 72. The other fixed contact of the potentiometer is grounded. A filter capacitor 82 is shunted across the potentiometer 72.

In a usual manner, the rectifier 78 rectifies the voltage appearing across the secondary of the power transformer 76. The rectifier voltage is filtered by the elements 80 and 82, and a positive direct voltage appears across the potentiometer 72. Then, by adjustment of the movable tap on the potentiometer 72, the proper positive direct exciting voltage can be supplied to the anode and screen grid of the pentode 64.

A half-wave rectifier tube 84 is connected to one side of the secondary 77 of the power transformer 76. This latter rectifier may be a simple diode whose cathode is connected to the secondary winding and whose anode is

connected to a choke coil 86. The choke coil, in turn, is connected to one of the fixed contacts of a potentiometer 88. The other fixed contact of the potentiometer 88 is grounded, and the potentiometer is shunted by a filter capacitor 90. The movable tap of the potentiometer 88 is connected to a resistor 92 which, in turn, is connected to the control grid of the gas discharge tube 20.

In known manner, a negative direct voltage is developed across the potentiometer 88, and this voltage is used to provide the appropriate adjustable bias for the gas discharge tube 20. This negative bias is controllable merely by shifting the movable tap on the potentiometer 88.

The voltage appearing across the secondary of the transformer 22 is shown, for example, in curve "A" in Figure 3. This voltage may be a usual 60-cycle alternating-current sinusoidal wave. The voltage across the secondary is introduced to the anode of the gas discharge tube 20. As is well known, the discharge tube 20 can be fired only on the positive half-cycles of this voltage wave, when the anode is driven positive with respect to the grounded cathode.

The pentode 64 is normally conductive so that a relatively low voltage appears at its anode. The phase shifting circuit 16 operates in known manner to produce a pair of signals which are mixed across the resistor 60.

One of the signals is phase shifted by the capacitor 54, and the other has an amplitude which is controllable by adjustment of the resistor 52. The result is a peaked complex wave across the resistor 60 whose peak may be shifted with respect to a time base merely by shifting the value of the resistor 52.

The negative half-cycle only of the complex wave across the resistor 60 is introduced to the control grid of the pentode 64 due to the action of the diode 58. In this manner, the pentode 64 may be periodically rendered non-conductive and at a point in each cycle of the complex wave, as determined by the adjustment of the resistor 52.

Each time the pentode 64 is rendered non-conductive, it introduces a positive triggering pulse to the control grid of the gas discharge tube 20. These triggering pulses are shown in the curve "B" of Figure 3. The peaks of the pulses of the curve "B" may be made to occur at any time during respective ones of the positive half-cycles of the curve "A" in Figure 3 under the control of the resistor 52, as noted above.

When each of the pulses of the curve "B" fires the gas discharge tube 20, the discharge of the tube continues during each triggering cycle until the corresponding cycle of the voltage wave of curve "A" introduced to its anode swings negative. This is in accordance with the well known triggering of thyratrons or other gas discharge tubes. The resulting plate voltage on the gas discharge tube 20 is shown in curve "C" of Figure 3, and the current pulses passed through the bath 10 of Figure 1 are shown in the curve "D." Merely by controlling the point of each positive half-cycle of the curve "A" at which the triggering pulses of the curve "B" trigger the gas discharge tube 20, the individual duration and amplitude of the pulses of curve "D" can be controlled. This is effectuated under the control of the resistor 52, as described above. This enables the characteristics of the current pulses passed through the bath 10 to be tailored to meet the needs of the material being processed at any particular time.

The effect on the current pulses through the bath as the control 52 is varied is shown in Figure 4. The curve A of Figure 4 shows the in phase condition whereby the current pulse is 100% of the positive half cycle of the voltage across the secondary of the transformer 22. The curve B of Figure 4 shows a condition similar to that of the curve D of Figure 3, in which the control 52 is varied so that current flows through the bath for about 50% of the positive half cycle. Finally, the curve C of Figure 4 shows the condition of the control 52 in which the current pulses flow through the bath at reduced amplitude and for a small percentage of the half cycles.

The curves of Figure 4 demonstrate the extreme flexibility of the system, and how the amplitude of the individual current pulses can be simply controlled, as well as the cooling intervals between successive ones of the pulses. Typical operation is represented by the condition of the curve B of Figure 4 in which current flows through the bath 10 for about 25% of the full cycle of voltage across the secondary of the transformer 22. This control may be carried out manually or automatically for the different substances to be anodized. Moreover, the control can be varied for optimum anodizing results during the anodizing process of any particular substance. An indication by a cathode-ray oscilloscope, or similar instrument, of the wave shape of the current pulses may serve as a convenient monitor of the desired condition of the anodizing current at any particular time.

The gaseous discharge tube 20 may have one or more tubes connected in parallel with it to increase the current capabilities of the system. Also, by connecting a pair of tubes such as the tube 20 in a known back-to-back circuit, and by the use of a tapped output transformer, negative current pulses can also be produced through the bath 10 in addition to the positive current pulses discussed above. These negative current pulses may be controlled to have a reduced amplitude, and they may serve further to reduce the effects of anode polarization.

The process of the invention offers a wider range of metallic alloys that can be anodized successfully. The process greatly reduces the possibility of burning the workpiece. In addition to this, the process increases the rate at which the anodic film is built up, as compared to the prior art processes.

The present invention provides, therefore, an improved anodizing process and apparatus in which the processing speed of the workpiece being anodized may be materially increased. This results in a harder anodic film because it is subject to the action of the electrolyte for a shorter length of time, as compared with the prior art processes.

Also, the apparatus and process of the invention provides for a cooling interval at the anode workpiece to permit an increase in current density further to enhance

the hardness characteristics of the anodic film formed at the anode and to increase the obtainable thickness of the film.

5 The refrigeration requirements of the system are materially reduced as compared to the prior art processes, this being due to the anode cooling by the pulsing action of the apparatus and process of the invention.

10 The actual electrical control system and components of the apparatus of the invention are relatively simple in their construction, and the individual circuits are in themselves simple to construct and they use well known component parts. The system is readily adjustable to fit the needs of any particular material or alloy being processed, and it is straight-forward and foolproof in its operation.

15 Also, the improved system and process of the invention is extremely economical and efficient in power consumption. A constructed embodiment of the invention, for example, was found to require essentially fifty percent of the amount of power required by a typical prior art system.

I claim:

20 1. An anodizing method for forming a relatively thick and hard inorganic corrosion-resistant non-reactive anodic film on an electrically conductive body capable of being anodized which includes: providing an electrolyte having a tendency to dissolve the anodic oxide film on the electrically conductive body, the rate of which dissolution increases with increase in the temperature of the electrolyte at the surface of the body, immersing at least a portion of the electrically conductive body in the electrolyte, and passing a series of uni-directional electrical current pulses of a repetition frequency of about 60 pulses per second through the electrolyte and through the electrically conductive body to provide an anodic oxide film on the electrically conductive body, with each successive pulse penetrating the oxide film to the electrically conductive body and with each of said unidirectional current pulses being separated by an interval of essentially zero current flow through the electrolyte and through the electrically conductive body, with the interval between each of such current pulses being of a duration approximately three times the duration of the interval of each of the current pulses to provide a cooling period at the surface of the immersed portion of the electrically conductive body between each of said current pulses, the cooling period between each current pulse being approximately three times the duration of each current pulse.

25 2. The method defined in claim 1 which further includes refrigerating the electrolyte to a temperature less than 45 degrees Fahrenheit.

30 3. An anodizing method of forming a relatively thick and hard inorganic corrosion-resistant non-reactive anodic film on an electrically conductive body capable of being anodized which includes: providing an electrolyte having a tendency to dissolve the anodic oxide film on the electrically conductive body, the rate of which dissolution increases with increase in the temperature of the electrolyte at the surface of the body, immersing at least a portion of the electrically conductive body in the electrolyte, and passing a series of uni-directional electrical current pulses of a selected repetition frequency through the electrolyte and through the electrically conductive body to provide an anodic oxide film on the electrically conductive body, with each successive pulse penetrating the oxide film to the electrically conductive body and with each of said pulses being separated by an interval of essentially zero current flow through the electrolyte and through the electrically conductive body, with the duration of each of such current pulses constituting up to approximately 25 percent of the total repetition period of such pulses to provide an interval between successive ones of the current pulses so as to establish a cooling period at the surface of the immersed portion of the

electrically conductive body between each of said current pulses.

4. An anodizing method for forming a relatively thick and hard inorganic corrosion-resistant non-reactive anodic film on an electrically conductive body capable of being anodized which includes: providing an electrolyte having a tendency to dissolve the anodic oxide film on the electrically conductive body, the rate of which dissolution increases with increase in the temperature of the electrolyte at the surface of the body, immersing at least a portion of the electrically conductive body in the electrolyte, and passing a series of uni-directional electrical current pulses of a selected repetition frequency through the electrolyte and through the electrically conductive body to provide an anodic oxide film on the electrically conductive body, with each successive pulse penetrating the oxide film to the electrically conductive body, with each of said pulses being separated by an interval of essentially zero current flow through the electrolyte and through the electrically conductive body, with the duration of each of such current pulses constituting approximately 25 percent of the total repetition period of such pulses to provide an interval between each such current pulses of a duration approximately three times the duration of the interval of each of the current pulses so as to establish a cooling period at the surface of the immersed portion of the electrically conductive body between each of said current pulses which is approximately three times the duration of each current pulse.

5. An anodizing method for forming a relatively thick and hard inorganic corrosion-resistant non-reactive anodic film on an electrically conductive body capable of being anodized which includes: providing an electrolyte having a tendency to dissolve the anodic oxide film on the electrically conductive body, the rate of which dis-

5  
10  
15  
20  
25

solution increases with increase in the temperature of the electrolyte at the surface of the body, immersing at least a portion of the electrically conductive body in the electrolyte, and passing a series of uni-directional electrical current pulses of a repetition frequency of about 60 pulses per second through the electrolyte and through the electrically conductive body to provide an anodic oxide film on the electrically conductive body, with each successive pulse penetrating the oxide film to the electrically conductive body and with each of said unidirectional current pulses being separated by an interval of essentially zero current flow through the electrolyte and through the electrically conductive body, with the duration of each of the current pulses constituting up to approximately 25 percent of the total repetition period of such pulses to provide an interval between each of such current pulses of a duration at least three times the duration of the interval of each of the current pulses so as to establish a cooling period at the surface of the immersed portion of the electrically conductive body between each of said current pulses which is at least twice the duration of each current pulse.

References Cited in the file of this patent

UNITED STATES PATENTS

|           |             |               |
|-----------|-------------|---------------|
| 2,396,685 | Coggins     | Mar. 19, 1946 |
| 2,541,275 | Odier       | Feb. 13, 1951 |
| 2,582,020 | Emery       | Jan. 8, 1952  |
| 2,692,851 | Burrows     | Oct. 26, 1954 |
| 2,715,095 | Cohn        | Aug. 9, 1955  |
| 2,726,203 | Rockafellow | Dec. 6, 1955  |

FOREIGN PATENTS

|         |               |               |
|---------|---------------|---------------|
| 636,665 | Germany       | Oct. 13, 1936 |
| 716,554 | Great Britain | Oct. 6, 1954  |